

## UNITED STATES PATENT OFFICE

2,657,139

## PROCESS OF REMOVING COLOR DEVELOPER STAIN IN AZINE DYE IMAGES

James E. Bates, Chenango Bridge, N. Y., assignor to General Aniline & Film Corporation, New York, N. Y., a corporation of Delaware

No Drawing. Application December 22, 1950,  
Serial No. 202,437

6 Claims. (Cl. 95—88)

1

This invention relates to photographic rinse baths for removing color developer stains from azine dyestuff images following color forming development with 2,4-diaminoaniline developing agents.

It is known that azine dyestuff images are produced by color developing silver halide emulsions containing azine color formers with a 2,4-diaminoaniline developing agent. The procedure of this process is fully described in U. S. P. 2,486,440.

Despite the many recognized advantages of this process, the 2,4-diaminoaniline developing agents employed therein possess one disadvantage which causes a somewhat serious problem. The disadvantage occurs in the development of the multi-layer color film of the azine type and is manifested especially when the aromatic triamino developing solution is old and badly oxidized by leaving a developer stain in the processed film. This stain in most cases is quite substantive to gelatin but can under certain circumstances be to some extent removed by excessively long water washing after color development. This developer stain is observed particularly in the highlights or whites of the processed film. In the color developed areas of the film, it produces a serious loss in color brilliance and a degradation of color rendition. Moreover, the developer contributes in no small degree to the loss of storage stability of the final color image, including both the so-called light, humidity, and heat fading characteristics.

In a multi-layer color film of the azine type which is composed of three layers colored yellow, magenta, and cyan, an ideal red reproduction would be composed of images wholly contained in the yellow and magenta layers and with a minimum of density in the cyan layer. Inasmuch as 2,4-diaminoanilines, as a general class, are oxidized quite readily by air and the residual color developing agent is oxidized by the bleaching steps subsequent to normal color development, an appreciable degradation of the red manifests itself by a stain density formed in the cyan layer.

To overcome the excessive washing time and the formation of stain, rinse baths consisting of aqueous solutions of water soluble open-chain mono-, di-, and tribasic acids, such as acetic, citric, maleic, etc., have been suggested. Short-stop baths containing these acids are, however, ineffective when applied to the azine process since they minimize the solubility of the 2,4-diaminoaniline color developers and lead to a product of extremely poor color rendition. Rinse baths of aqueous solutions of aliphatic aldehydes

2

and diketones, such as formaldehyde, paraformaldehyde, and the like, have also been proposed but these are also ineffective since a falsification of color occurs.

It is an object of the present invention to provide a simple and economical method of eliminating color stain and degradation from azine dyestuff images obtained by color forming development with 2,4-diaminoaniline developing agents. Other objects and advantages will appear hereinafter.

The above objects are accomplished by treating an azine multilayer color film, after color forming development with an aqueous rinse bath containing from 0.1 to 10% of formaldehyde and from 0.1 to 10% of a water-soluble acid, such as hydrochloric, phosphoric, acetic, maleic, citric, acrylic, oxalic, tartaric, and the like. The pH of the resulting rinse bath is immaterial and in these concentrations, and in the presence of formaldehyde, the acid does not form an insoluble complex with the residual 2,4-diaminoaniline developing agent retained by the film, i. e., does not precipitate it upon the film or in the layers thereof. The presence of the water-soluble acid tends to cause the formaldehyde to form a water-soluble 2,4-diaminoaniline-formaldehyde complex which is readily washed from the emulsion by one or two water rinses after the processing steps have been completed.

The 2,4-diaminoanilines which are utilized as the color developers for the production of azine dyestuff images are of the type described in the aforementioned Patent 2,486,440 and in application Serial No. 101,913, filed June 28, 1949, now Patent No. 2,570,116, and entitled "Color Developers for the Production of Azine Dye Images."

Specific examples of such developing agents are:

- 40 4-( $\beta$ -hydroxyethylamino)-6-(4'-carboxymethoxyphenylamino)-metanilic acid
- 41 4-(carboxymethylamino)-6-(4'-methoxyphenylamino)-metanilic acid
- 42 2-( $\beta$ -sulfoethylamino)-4-phenylamino aniline
- 43 4,6-di( $\beta$ -hydroxyethylamino)-metanilic acid
- 44 4-( $\beta$ -hydroxyethylamino)-6-phenylamino-metanilic acid
- 45 2-( $\beta$ -hydroxyethylamino)-4-( $\beta$ -sulfoethylamino)-5-methyl aniline
- 46 4-( $\beta$ -hydroxy- $\beta$ -methylethylamino)-6-phenylamino-metanilic acid
- 47 4-[ $\alpha$ -di(hydroxyethyl)ethylamino]-6-(3'-ethoxyphenylamino)-metanilic acid
- 48 4-( $\beta$ -hydroxyethylamino)-6-methylamino-metanilic acid

- 4-(sulfomethylamino) - 6 - methylphenylamino-metanilic acid  
 4-( $\beta$  - hydroxyethylamino) - 6 - methylamino-metanilic acid

Color formers which are used with the aforementioned developers to give yellow azine dye images are also described in the aforementioned application Serial No. 101,913. These compounds are typified by the fact that they are open-chain ketomethylene compounds. Examples of such compounds are:

- Acetoacetanilide  
 N-1-naphthylacetooacetamide  
 N,N'-ethylenbisacetooacetamide  
 p,p'-bi-o-aceacetanilide  
 N-2-naphthylbenzoylacetamide  
 p,p'-bi-aceacetanilide  
 a,a'-terephthaloylbis-(3-chloro-4,6-dimethoxyacetanilide)  
 a-benzoylacetanilide

Preferably, the color formers utilized contain a group rendering them non-migratory in the emulsion. Examples of such compounds are:

- 2-(m-benzoylacetamidophenyl)-1-octadecyl-5-benzimidazolesulfonic acid  
 3,3'-ureylenebis-5-p-benzoylacetamidobenzamide-benzenesulfonic acid  
 2-p-benzoylacetamidobenzamido-6-stearoyl-amino-p-toluenesulfonic acid  
 2-(p-benzoylacetamidophenyl)-1-octadecyl-5-benzimidazolesulfonic acid  
 p-cyanoacetyl-3-octadecenylsuccinalic acid.

Color formers capable of producing magenta dyestuff images are also described in the above identified application and in USP 2,524,741. Preferably, these color formers are 6-halogen-8-hydroxyquinolines, and particularly those which are non-migratory in the emulsions. Examples of the latter type compounds are:

- 6-stearoylamino-2-(2'-phenyl-6'-bromo-8'-hydroxycinchoninoyl)-aminotoluene-4-sulfonic acid  
 2-phenyl-6-chloro-8-hydroxycinchoninoyloctadecyl taurine  
 6-deoxy-3-(2-phenyl-6-bromo-8-hydroxycinchoninoyl)-amino-benzenesulfonic acid.  
 2-(3-stearoylaminophenyl)-6-bromo-8-hydroxycinchoninic acid  
 2-stearoylamino-6-(6-chloro-8-hydroxycinchoninoyl)-aminotoluene-4-sulfonic acid, and the like.

Color formers for the cyan image are also described in USP 2,570,116, issued October 2, 1951, and in USP 2,445,252, issued July 13, 1948. Preferably, these color formers are aryl-J-acid derivatives, particularly those containing a group rendering the color former non-migratory in the emulsion. Examples of the latter compounds are:

- dodecyl urethane of  $\beta$ -sulfoethyl-J-acid  
 tetradecyl urethane of p-anisyl-J-acid  
 2-hexadecyl urethane of phenyl-J-acid  
 4-stearoylamino-J-acid, and the like.

By employing an acidified formaldehyde solution, a substantial improvement in color brilliance and rendition is obtained. This is attributable to the fact that formaldehyde forms a highly soluble complex with the color developer in an acid solution, and as a consequence, reduces

color degradation and leads to improved color brilliance.

The following examples describe in detail the method for accomplishing the above objects. It is to be understood, however, that they are exemplary only and they are not to be construed as being limitative.

*Example I*

- 10 A red sensitive emulsion containing phenyl-J-acid-N-octadecyl urethane was exposed and the latent image developed in a black and white developer, re-exposed, and the residual silver halide developed in a solution of the following composition:

|                                                              | Grams |
|--------------------------------------------------------------|-------|
| Sodium carbonate (monohydrate)                               | 40    |
| Sodium sulfite                                               | 40    |
| Sodium sulfate                                               | 50    |
| Ethylenediamine                                              | 15    |
| 2-aminopyridine                                              | 10    |
| 4-( $\beta$ -hydroxyethylamino)-6-methylamino-metanilic acid | 5     |
| Water to make 1000 cc.                                       |       |

- 25 After color development, the layer was rinsed, and treated for 5 minutes in a bath of the following composition:

|                                        | grams |
|----------------------------------------|-------|
| Hydrochloric acid                      | 5     |
| Formaldehyde (40% aqueous solution) cc | 10    |

30 Water to make 1000 cc.

The film was washed, bleached in a ferricyanide bleach, and fixed in an acid hardening solution. There is obtained a cyan positive dye image completely free from stain and stable against accelerated adverse storage conditions.

*Example II*

- 40 An integral tripack with a bottom layer composed of a red sensitive emulsion containing phenyl-J-acid-N-octadecyl urethane, a middle layer composed of a green sensitive emulsion containing 2-stearoylamino-6-(8-hydroxycinchoninoylamino)-toluene-4-sulfonic acid, and a top layer composed of a blue sensitive emulsion containing 2-(4-benzoylacetaminophenyl)-1-octadecyl-5-benzimidazolesulfonic acid, was exposed and the latent image developed in a black and white developer, short-stopped, re-exposed, and the residual silver halide developed in a solution of the following composition:

|                                                              | Grams |
|--------------------------------------------------------------|-------|
| Sodium carbonate (monohydrate)                               | 40    |
| Sodium sulfite                                               | 60    |
| Potassium bromide                                            | 5     |
| Pyridine                                                     | 16    |
| Benzylamine                                                  | 1     |
| 4-( $\beta$ -hydroxyethylamino)-6-phenylamino-metanilic acid | 5     |
| Water to make 1000 cc.                                       |       |

55 After color development, the film was rinsed and treated for 5 minutes in a bath of the following composition:

|                                        | grams |
|----------------------------------------|-------|
| Acetic acid                            | 10    |
| Formaldehyde (40% aqueous solution) cc | 40    |

Water to make 1000 cc.

60 Water to make 1000 cc.

70 The film was washed, bleached in a ferricyanide bleach, and fixed in an acid hardening fixer solution. There was obtained a multicolor film containing stain-free positive dye images of excellent brilliance and freedom from color degradation.

## Example III

An integral tripack of essentially the same composition as in Example II was exposed and color developed for 15 minutes to a negative image in a solution of the following composition:

|                                                                  | Grams |
|------------------------------------------------------------------|-------|
| Trisodium phosphate                                              | 40    |
| Sodium sulfite                                                   | 40    |
| Potassium bromide                                                | 12.5  |
| Hydroxylamine hydrochloride                                      | 1     |
| 4-( $\beta$ -hydroxyethylamino)-6-benzylamino-<br>metanilic acid | 6     |
| Water to make 1000 cc.                                           |       |

After development, the film was rinsed and treated in a bath of the following composition:

|                                     |       |    |
|-------------------------------------|-------|----|
| Citric acid                         | grams | 10 |
| Formaldehyde (40% aqueous solution) | cc    | 20 |
| Water to make 1000 cc.              |       |    |

The film was washed, bleached in a ferricyanide bleach, and fixed in an acid hardening hypo solution. There was obtained a brilliant negative dye image completely free from stain and color degradation. The negative did not acquire additional stain nor become subject to color degradation during three weeks' accelerated aging at 90% relative humidity and 120° F.

It will be obvious to any one skilled in the art that many modifications, such as substituting equivalent materials and varying the proportions of materials used, are within the spirit and scope of the invention as defined in the appended claims.

## I claim:

1. In the process of eliminating stain in the production of subtractively colored azine dye images in a silver-halide emulsion involving exposure of said emulsion, color developing the same in a 2,4-diaminoaniline developer in the presence of a color former to produce a subtractively colored azine dye image, bleaching, fixing and washing said emulsion, the improvement which comprises interpolating between the color development and bleaching step a rinsing of the color developed emulsion with an aqueous solution containing from 0.1 to 10% of formaldehyde and 0.1 to 10% of a water soluble acid.
2. The process according to claim 1 wherein the acid is acetic.
3. The process according to claim 1 wherein the acid is hydrochloric.
4. The process according to claim 1 wherein the acid is maleic.
5. The process according to claim 1 wherein the acid is citric.
6. The process according to claim 1 wherein the acid is acrylic.

JAMES E. BATES.

## References Cited in the file of this patent

## UNITED STATES PATENTS

| Number    | Name   | Date          |
|-----------|--------|---------------|
| 2,367,548 | Vittum | Jan. 16, 1945 |
| 2,515,121 | Harsh  | July 11, 1950 |
| 2,518,686 | Harsh  | Aug. 15, 1950 |